

Feb. 9, 1937.

C. P. DEBUCH ET AL

**2,069,875**

# PROCESS OF AND APPARATUS FOR ROASTING ORES

Filed Sept. 11, 1934



*Inventor:*  
**CARL PAUL DEBUCH**  
**ERNST MARKWORTH**

34

A. J. Deller  
Attorney

## UNITED STATES PATENT OFFICE

2,069,875

PROCESS OF AND APPARATUS FOR  
ROASTING ORES

Carl Paul Debuch and Ernst Markworth, Frankfort-on-the-Main, Germany, assignors to American Lurgi Corporation, New York, N. Y., a corporation of New York

Application September 11, 1934, Serial No. 743,510  
In Germany March 10, 1934

11 Claims. (Cl. 263—33)

The present invention relates to the roasting of ores and more particularly to a process of roasting ores in rotary tube-furnaces and to an improved apparatus therefor.

5 It is known that the roasting of ores and other metallurgical materials in rotary tube-furnaces was confronted with certain difficulties which interfered very materially with the conditions essential to good roasting and with the operation of the apparatus. The main difficulties were 10 due to the exothermic nature of the roasting reactions which caused the temperature to become excessively high, especially in certain zones of the furnace, and brought about detrimental fusing 15 of the charge, which resulted in the formation of agglomerations and incrustations thereof in the interior of the furnace. As a result of the excessive heat and of the fusing of the charge, the inside lining of the furnace and other parts 20 of the furnace deteriorated rapidly. The agglomerations and incrustations, moreover, interfered with the operations of the apparatus and required frequent and expensive shut-downs and 25 repairs.

25 Various attempts were made to avoid the disadvantages noted hereinabove, but none, as far as it is known, was wholly successful and satisfactory in actual practice. Thus, for instance, instead of introducing the entire amount of the oxidizing air at one end of the furnace, the air was admitted through a number of nozzles evenly distributed over the entire length of the furnace. While this procedure brought about a more uniform temperature distribution, it did not prevent 30 excessive rising of the temperature and did not eliminate the fusing of the charge and the formation of agglomerations and incrustations. It was attempted to withdraw the excess heat from the furnace by increasing the air supply above the 35 normal amount essential for good roasting conditions, or by returning cooled exhaust gases to the furnace. This procedure, however, was found to be objectionable, because it detrimentally affected the roasting reactions and other conditions essential to good roasting. Furthermore, by increasing the volume of the outgoing gases, it also increased the dust carrying capacity thereof. In prior processes, it was necessary to operate the rotary tube-furnaces at low capacity, and reduce the rate at which the material was 40 being treated in order to prevent excessive rises in temperature causing sintering and agglomeration of the charge.

45 It is an object of the present invention to provide a process which substantially eliminates the

difficulties and shortcomings noted hereinabove, which is simple, practical and efficient, and which is capable of being carried into practice satisfactorily and economically.

5 It is another object of the invention to provide an improved process of roasting ores and other metallurgical materials in rotary tube-furnaces, which substantially prevents detrimental fusing and agglomeration of the charge, and which permits the rotary tube-furnaces to be operated at 10 a higher capacity than it has been possible heretofore.

The invention contemplates a method of withdrawing excess heat developed in the roasting apparatus without substantially disturbing the 15 conditions essential to good roasting.

A further object of the invention is to provide a process that will permit a higher concentration of  $\text{SO}_2$  gases in the furnace atmosphere than it has been possible heretofore in rotary tube-furnaces.

20 It is likewise within the contemplation of the invention to provide a simple and improved apparatus capable of carrying the present invention into practice successfully and economically.

25 The invention further provides special means for withdrawing heat developed in the roasting apparatus, according to the principle of the invention.

30 Other objects and advantages of the invention will become apparent from the following discussion taken in conjunction with the accompanying drawing in which:—

35 Fig. 1 shows diagrammatically a side elevational view, partly in section, of a preferred form of an apparatus embodying the present invention; and

Fig. 2 illustrates a longitudinal section of an air nozzle on a large scale.

40 In general, the invention comprises withdrawing heat from the furnace atmosphere and balancing the heat thus abstracted by increasing the charge of the material undergoing treatment. The heat is withdrawn in quantities sufficient to prevent substantially sintering and incrustations of the charge. According to the invention, withdrawal of heat may be effected by admitting the oxidizing air through a plurality of air-nozzles projecting into the furnace, and in addition by withdrawing heat from the walls 45 of the nozzles.

45 Referring more particularly to Fig. 1, the drawing illustrates by way of example, a rotary tube-furnace comprising a shell 1 lined with refractory material 2. Inlet and outlet means for 50

the material undergoing treatment are designated by reference characters 3 and 4 respectively. An outlet for the furnace gases is provided by exhaust gas flue 5 at the feed end of the furnace. 5 The apparatus is supported on track rings 6 and may be rotated through gear drive 7 by any conventional driving mechanism (not shown in the drawing).

A controllable amount of roasting air is admitted into the furnace through a plurality of air nozzles and distributed over the entire length of the furnace. The nozzles are mounted on shell 1 by means of an intermediate member 14, and are extended into the furnace to a sufficient depth to prevent the material treated in the furnace from reaching the outlet orifices of the nozzles. The nozzles consist substantially of an inner nozzle-tube 11 and a jacket tube 10. Interspaced between the jacket and tube 11 is another tube 12 which preferably does not extend entirely to the outlet end of the nozzle. An inlet for the roasting air is provided at the nozzle head 15. Reference character 13 denotes a connection for a cooling medium for the air nozzle. 25 A suitable cooling medium for the nozzles may be air, which may be supplied by a blower 19 through pipe 18, distributor head 17 and pipes 16 which rotate with the furnace and are provided with control devices 9. The cooling air flows through connections 13 into the space between tubes 11 and 12 to the end of the nozzle where it is deflected into the outer jacket and flows back between tubes 12 and 10 to outlet 20 at the nozzle head.

35 The roasting air is admitted into the furnace through pipe 11. If the furnace operates under negative pressure, pipe 11 may be open at both ends and the roasting air is drawn in the furnace directly from the outside. In order to control 40 the flow of air, the outer end of pipe 11 at the nozzle head may be provided with valves, dampers, or similar controlling devices. The roasting air, however, may be supplied also under pressure. For example, the nozzle tubes 11 may be 45 controllably connected to blower 19 supplying the cooling air for the nozzles.

Referring more particularly to Fig. 2, wherein a preferred embodiment of a suitable air nozzle is shown more in detail, reference character 14 50 indicates an intermediate annular member, for example, a cast-steel ring, which may be secured to iron shell 1 of the furnace by means of screws or rivets. Fixed on intermediate member 14, for instance by means of bolts is nozzle head 15, 55 which may comprise annular members 15a, 15g, a sealing member 15b and an air damper 15c, assembled to form two annular spaces 15d and 15f which are not in direct communication with each other. Damper 15c may be of the usual type employed for controlling the flow of air in the nozzles hitherto in use.

60 The outer tube 10 of the nozzle is suitably secured to intermediate member 14, for instance by clamping the flared end thereof between ring 65 15a and intermediate member 14. At the discharge end of the nozzle, tube 10 is joined to the end of tube 11 to make a substantially air tight connection, for instance by welding. The other end of tube 11, however, is preferably not fastened and may be only made to fit closely into the central bore of annular member 15a, thereby 70 allowing for free thermal expansion of the tubes. At the intake end of the nozzle, inner tube 12 may be suitably joined to wall 15g between annular spaces 15d and 15f. The other end of the

tube, however, is preferably left free in order to allow for thermal expansion and provide a passage for cooling air between inner jacket 8a and outer jacket 8b of the nozzle at the outlet end thereof. 5

The nozzle head may be made of cast iron, bronze, aluminum, or similar material. Materials suitable for the nozzle tubes may be, for instance, iron, copper or heat resisting alloys. It is preferable to use heat resisting steel or alloys, 10 because, due to their excellent durability in service, thinner gauge material can be used, and the nozzles will be lighter than if other material is used. It is to be observed, however, that it may be sufficient to have only outer tube 10 made of 15 heat-resisting alloys while a less expensive material may be employed for tubes 11 and 12, which in service are usually maintained by the cooling to a substantially low temperature. In view of the fact that inner tube 11 is cooled to a lower temperature than tubes 10 and 12, it may be advisable 20 to construct the nozzle so that tube 11 takes up the principal mechanical stresses and also carry tubes 12 and 10. It is possible, however, to distribute the stresses in a suitable manner among 25 all three tubes.

In carrying the present invention into practice, a proper amount of roasting air is admitted into furnace 1 rotating at a suitable rate. A predetermined amount of the material to be roasted, is 30 charged through charging device 3. As the material undergoing treatment travels toward outlet 4 at the other end of the furnace, it is ignited and subjected to the oxidizing action of the roasting air which attacks the sulphides and brings 35 about other desired chemical changes of the charge.

It is to be observed that, due to the exothermic nature of the roasting reaction, the temperature of the charge tends to be raised rapidly and, if 40 left uncontrolled, some of the unroasted material will fuse together or "matte" causing agglomerations and incrustations of the mass, and the roasting operation will be interfered with, perhaps stopped altogether. 45

It was found, however, that if the air nozzles projecting into the furnace are internally cooled according to the principle of the invention, the temperature can be controlled substantially to prevent fusing of the charge. The herein described method employed for cooling the nozzles may extensively be controlled and adapted to suit the working conditions in the several zones of the furnace, by intensifying or diminishing the cooling, or by entirely suppressing the cooling of individual nozzles. If some of the furnace zones become too cold, the heated cooling air from other nozzles may be employed as roasting air in such zones. The temperature of the furnace may be controlled to maintain substantially the desirable 60 conditions in the furnace. 55

It is possible to abstract by the aforesaid method large quantities of heat which it is to be observed is withdrawn substantially all from the furnace gases. It has been determined that of 65 the heat generated in the furnace by the roasting reactions, approximately 50% is contained in the furnace gases. By properly controlling the cooling of the air nozzles according to the invention, it is possible to withdraw approximately 50% of the 70 heat in the furnace gases, or about 25% of the total heat generated in the furnace. The heat thus removed may be balanced by treating a correspondingly larger amount of material which in roasting will develop heat 25% in excess of the 75

normal charge. In some cases, however, it may be advisable to increase the charge so as to replace only 15% of the heat withdrawn by cooling. In this case, with the intensity of cooling a high concentration of sulphur dioxide in the furnace gases may be obtained, for instance, 13% or over.

The cooling of the nozzles can be effected by means of gases or liquids, for instance, air, steam, 10 or water. Water cooling is especially effective and is preferable when large quantities of heat are to be withdrawn from the furnace, or when comparatively small cooling surfaces are available. On the other hand, cooling with gases such as 15 air, has the advantage that condensations on the outer surface of the nozzle are substantially prevented. Furthermore, the cooling air, which has been heated in passing through the nozzle, may be utilized for heating or drying, or similar purposes.

It is to be observed that the present invention provides a process whereby ores and other metallurgical materials may be roasted efficiently without substantially disturbing the desired conditions 25 essential to good roasting, and whereby the efficiency of rotary tube-furnaces may be increased without, however, causing fusing and incrustations of the charge.

It is to be noted that since the heat is withdrawn substantially all from the atmosphere of the furnace and not from the material undergoing treatment, substantially little adverse influence is exerted on the roasting reactions, and active 30 roasting may thereby be maintained without, however, causing overheating of the charge.

It is also to be observed that the cooling is effected within the furnace without, however, diluting, contaminating, or otherwise changing the composition of nature of the furnace atmosphere. 40 The amount of roasting air entering the furnace can thereby be controlled to give the most active roasting atmosphere, and other conditions such as the rate of removal of the furnace gases, may be adjusted to effect efficient roasting of the 45 charge.

Furthermore, the invention provides for an efficient and controlled withdrawal of heat which may be partly balanced by increasing the rate at which the material is being treated, thereby 50 increasing the efficiency of the furnace. As more fully disclosed hereinabove, this also results in a higher concentration of sulphur dioxide in the furnace atmosphere than it has been possible heretofore in rotary tube-furnaces.

Although the present invention has been described in conjunction with preferred embodiments, it is understood that modifications and variations may be resorted to without departing 55 from the spirit of the invention, as those skilled in the art will readily understand.

We claim:—

1. The process of roasting ores in a rotary tube-furnace and of controlling the reaction temperature in said furnace which comprises passing ore to be roasted through a rotary tube-furnace, admitting roasting air into said furnace as a plurality of jets at spaced intervals of the length thereof, discharging said roasting air substantially radially into zones adjacent to the axis of the furnace, circulating a cooling medium within the furnace in association with each of said jets of roasting air but independently thereof, and withdrawing said cooling fluid, whereby heat is withdrawn from the gases in the furnace and the

roasting air is discharged into the furnace in a substantially cool state.

2. The process of roasting ores in a rotary tube-furnace and of controlling the reaction temperature in said furnace which comprises passing ore to be roasted through a rotary tube furnace, admitting roasting air into said furnace as a plurality of jets at spaced intervals of the length thereof, discharging said roasting air substantially radially to the sides of said furnace into 5 zones adjacent to the axis of the furnace, circulating cooling air within the furnace in association with substantially the entire length of each of said jets of roasting air but independently thereof, withdrawing said cooling air to withdraw 10 heat from the gases in the furnace and to discharge roasting air into the furnace in a substantially cool state, and separately controlling the amount of cooling air circulated within separate zones of the furnace to control the temperature 15 independently in said zones.

3. The process of roasting ores in a rotary tube-furnace and of controlling the reaction temperature in said furnace which comprises passing ore to be roasted through a rotary tube furnace, 25 admitting roasting air into said furnace as a plurality of jets at spaced intervals of the length thereof, discharging said roasting air substantially radially to the sides of said furnace into zones adjacent to the axis of the furnace, 30 circulating cooling air within the furnace in association with substantially the entire length of each of said jets of roasting air but independently thereof, withdrawing said cooling air to withdraw heat from the gases in the furnace and 35 to discharge roasting air into the furnace in a substantially cool state, and balancing the heat thus abstracted by increasing the charge of the ore undergoing treatment.

4. The process of roasting ores in a rotary tube-furnace and of controlling the reaction temperature in said furnace which comprises passing ore to be roasted through a rotary tube furnace, admitting roasting air into said furnace as a plurality of jets at spaced intervals of the length 45 thereof, discharging said roasting air substantially radially to the sides of said furnace into zones adjacent to the axis of the furnace, circulating cooling air within the furnace in association with substantially the entire length of 50 each of said jets of roasting air but independently thereof, withdrawing said cooling air to withdraw heat from the gases in the furnace and to discharge roasting air into the furnace in a substantially cool state, controlling the amount of cooling air circulated within the furnace to withdraw 55 substantially 50% of the heat contained in the furnace gases, and replacing heat thus abstracted from the furnace gases by increasing the charge of the ore undergoing treatment substantially 60 15%.

5. A rotary tube furnace for roasting ores comprising a rotatable shell, means for charging material to be treated into said shell and for withdrawing treated material therefrom, a plurality 65 of air nozzles for supplying roasting air to the interior of said shell, said air nozzles being distributed at spaced intervals over said shell and extending therethrough to a substantial depth in the interior thereof, an outer jacket in intimate 70 heat exchange with the furnace gases surrounding substantially the entire length of each of said air nozzles, means for circulating a cooling fluid within said jacket for withdrawing substantial quantities of heat from said furnace gases to 75

maintain their temperature within preferred limits, and means for withdrawing combustion gases from the furnace.

6. A rotary tube furnace for roasting ores comprising a rotatable shell, means for charging material to be treated into said shell and for withdrawing treated material therefrom, a plurality of air nozzles for supplying roasting air to the interior of said shell, said air nozzles being distributed at spaced intervals over said shell and extending therethrough to a substantial depth in the interior thereof, an outer jacket in intimate heat exchange with the furnace gases surrounding substantially the entire length of each of said air nozzles, means for circulating a cooling fluid within said jacket for withdrawing substantial quantities of heat from said furnace gases to maintain their temperature within preferred limits, means for supplying said cooling fluid to said jackets, and means for withdrawing combustion gases from the furnace.

7. A rotary tube furnace for roasting ores comprising a rotatable shell, means for charging material to be treated into said shell and for withdrawing treated material therefrom, a plurality of air nozzles for supplying roasting air to the interior of said shell, said air nozzles being distributed at spaced intervals over said shell and extending therethrough to a substantial depth in the interior thereof, an outer jacket in intimate heat exchange with the furnace gases surrounding substantially the entire length of each of said air nozzles, means for circulating a cooling fluid within said jacket for withdrawing substantial quantities of heat from said furnace gases to maintain their temperature within preferred limits, a blower for supplying cooling fluid to said jackets and conduit means mounted on said shell for connecting said blower to said jackets.

8. The process of roasting ores in a rotary tube furnace and of controlling the reaction temperature in said furnace which comprises introducing roasting air into the interior of a rotary tube furnace through a plurality of air nozzles projecting into the furnace at spaced intervals, discharging said roasting air substantially radially into zones adjacent to the axis of the furnace, circulating a stream of a cooling fluid in indirect and intimate heat exchange with each of said streams of roasting air and with said furnace gases, and continuously withdrawing said cooling fluid whereby heat is withdrawn from said furnace gases and the temperature of said roast-

ing air and of said furnace gases is maintained within preferred limits.

9. The process of roasting ores in a rotary tube furnace and of controlling the reaction temperature in said furnace which comprises introducing roasting air into the interior of a rotary tube furnace in a plurality of streams at spaced intervals, discharging said roasting air substantially radially into zones adjacent to the axis of the furnace, circulating a stream of cooling fluid in indirect and intimate heat exchange with each of said streams of roasting air and with said furnace gases, independently controlling each of said streams of cooling fluid, and continuously withdrawing said cooling fluid whereby heat is withdrawn from said furnace gases and the temperature of said roasting air and of said furnace gases is maintained within preferred limits.

10. The process of roasting ores in a rotary tube furnace and of controlling the reaction temperature in said furnace which comprises introducing roasting air into the interior of a rotary tube furnace in a plurality of streams at spaced intervals, discharging said roasting air into zones adjacent to the axis of the furnace, circulating a stream of cooling fluid in indirect and intimate heat exchange with each of said streams of roasting air and with said furnace gases, independently controlling each of said streams of cooling fluid, and continuously withdrawing said cooling fluid whereby heat is withdrawn from said furnace gases and the temperature of said roasting air and of said furnace gases is maintained within preferred limits.

11. The process of roasting ores in a rotary tube furnace and of controlling the reaction temperature in said furnace which comprises introducing roasting air into the interior of a rotary tube furnace in a plurality of streams at spaced intervals, discharging said roasting air into zones adjacent to the axis of the furnace, circulating a stream of cooling air in indirect and intimate heat exchange with a selected plurality of said streams of roasting air and with said furnace gases, independently controlling each of said streams of cooling air, continuously withdrawing said cooling air whereby heat is withdrawn from said furnace, and reintroducing said withdrawn cooling air as roasting air into the cooler zones of said furnace to maintain preferred temperatures therein.

CARL PAUL DEBUCH.  
ERNST MARKWORTH.